

# UNITED STATES PATENT OFFICE.

EPES E. ELLERY AND JOSEPH F. ELLERY, OF NEW YORK, N. Y.

## IMPROVEMENT IN WATER-PROOF PAINTS.

Specification forming part of Letters Patent No. 24,620, dated July 5, 1859.

*To all whom it may concern:*

Be it known that we, EPES E. ELLERY and JOSEPH F. ELLERY, both of the city, county, and State of New York, have invented a certain new and useful Water-Proof Paint; and we do hereby declare that the following is a full and exact description of the materials used in and the process of compounding the same.

The nature of our invention consists in combining the materials hereinafter described, in the proportions set forth, for the purpose of producing a paint to withstand and resist the effects of wet, moisture, and vapor.

To enable others skilled in the art to compound and produce our water-proof paint, we will proceed to describe its constituent materials and the process by which we combine and compound them.

We take twelve pounds of india-rubber, either in its crude form, or refuse or scrap manufactured rubber, and dissolve it by heat in six gallons of linseed-oil. We then take twelve pounds of gutta-percha, either in its crude form or refuse scraps that have been manufactured, and dissolve it by heat in twelve gallons of linseed-oil. These articles are then mixed together, and into the mixture thus obtained we put three gallons of shellac varnish, made by dissolving six pounds of gum-shellac in three gallons of alcohol; and the mixture is then thoroughly incorporated by stirring them by mechanical or other means. From two and one-half to three and one-half gallons of this mixture, according to the required thickness of the coating, is then mixed with one hundred pounds of coloring-matter, either Spanish brown, ocher, Venetian red, or other material, according to the color required to be produced, by passing the mixture through a paint-mill in the ordinary manner, and the paint is then ready for use. The india-rubber in the mixture gives to it a proper elasticity to prevent the paint being injured by the changes of the atmosphere from heat to cold,

and, with the gutta-percha and shellac varnish, forms a coating, when dried upon the surface to which it is applied, which is completely impervious to water and is unaffected by vapor, moisture, or dampness. The gutta-percha is a well-known non-conductor of heat, and tends to prevent the paint being injured by the changes of temperature, while the shellac varnish, when the paint is dried, forms a hardened coat which resists the effects of wet and dampness, and which, in combination with the other ingredients in the composition, loses its liability to crack and break when subjected to changes of temperature. The india-rubber and gutta-percha are dissolved in the linseed-oil separately, for the reason that they will not combine together as thoroughly and effectually with the oil when mixed together as when they are dissolved separately, as described, and then mixed together.

This paint is applicable to the covering of all exposed surfaces, but is peculiarly applicable to the covering of exposed iron structures, which are peculiarly liable to be oxidized by wet, vapor, or moisture, as it forms a coating upon such surfaces which effectually resists the effects of changes of temperature and of wet and moisture, and which preserves such surfaces for a longer period than any of the paints in common use.

We do not claim the use of the materials herein described separately, as they have been used before for different purposes.

What we claim as our invention, and desire to secure by Letters Patent, is—

The composition prepared and composed of the materials, as described, in the proportions set forth, for the purpose of making water-proof paint.

EPES E. ELLERY.  
JOSEPH F. ELLERY.

Witnesses:

M. HASKELL,  
GEORGE N. BUCKMAN.